

## 1

3,692,589

### METHODS FOR REDUCING WEAR AND SEIZURE BETWEEN RUBBING TITANIUM AND STEEL SURFACES

Arthur M. Shapiro, Philadelphia, Pa., assignor to the United States of America as represented by the Secretary of the Army  
No Drawing. Filed Nov. 19, 1970, Ser. No. 91,155  
Int. Cl. C23f 1/00

U.S. Cl. 148—6

6 Claims

#### ABSTRACT OF THE DISCLOSURE

Processes for improving wear and seizure resistance between high speed rubbing titanium and steel surfaces by reacting the titanium initially with sodium fluoride at elevated temperatures over an extended period, the metal surfaces being lubricated with a dialkyldithiophosphate.

The invention described herein may be manufactured, used and licensed by or for the Government for governmental purposes without the payment to me of any royalty thereon.

This invention relates to lubricating processes and more particularly concerns methods for improving wear and seizure resistance between high speed rubbing titanium and steel surfaces.

Wear between titanium and steel surfaces poses a particularly severe lubrication problem, due in part to the well known fact that titanium readily galls and seizes. Methods to improve wear and seizure resistance between these metals have met with limited success and are accompanied with attendant disadvantages. For example, titanium has been coated with fluoride-phosphate by immersing a titanium piece into a solution thereof. A molybdenum disulphide-resin layer was then bound thereto by appropriate heat treating steps. The resin most commonly employed was a condensation product of bisphenol A and epichlorohydrin. The process was costly and time-consuming, requiring a two-layer system.

Another method for reducing wear and seizure involving titanium pieces required the formation of an alloy

## 2

concentration gradient at or near the titanium surfaces which would contact the steel surfaces. The alloying constituent was commonly a noble metal such as gold or silver, both of which are very costly.

Other methods were ineffective, unreliable, or could not be adequately reproduced for satisfactory industrial applications.

It is therefore an object of this invention to provide improved methods for treating titanium pieces to thus permit their satisfactory use when subjected to rubbing against steel, especially at high speeds.

Other and further objects of the invention will be apparent to those skilled in the art upon study of this disclosure.

In accordance with the above objects, I have discovered that titanium pieces immersed in sodium fluoride at elevated temperatures for extended periods are capable of withstanding high speed rubbing contact with certain steels when appropriate lubricants are used therewith.

More specifically, I have discovered that when 75A titanium is immersed in NaF at elevated temperatures for several hours, that wear and seizure resistance of the titanium is remarkably improved when contacting or rubbing 52100 or AISI 1137 steels when appropriate lubricants are present.

Anti-wear data were obtained using the Shell 4-Ball Wear Tester, described in an article by G. D. Boerlage, Engineering, vol. 136 (1933), page 46 et seq.

Anti-seizure data were obtained using the well-known Falex Extreme Pressure Tester described in Lubrication Engineering, September 1946, V. A. Ryan.

The Falex tests were conducted using jaw blocks made from AISI 1137 steel, R<sub>c</sub>20 and the pin made from 75A titanium. The jaw load was increased from 0 to 250 pounds by engaging the eccentric arm of the ratchet wheel. When the jaw load reached 250 pounds, the eccentric arm was disengaged and the load maintained for one minute. Using the same procedure, the jaw load was increased in increments of 250 pounds until failure occurred. The pin rotated at 290 r.p.m.

The 4-Ball Wear tests were conducted at 1200 r.p.m. at room temperature. The upper ball was 52100 steel, 1/2 inch in diameter, while the lower balls were 75A titanium of the same diameter. Results of tests are presented below:

#### ANTI-WEAR AND ANTI-SEIZURE DATA<sup>a</sup> OBTAINED WITH RUBBING TI AND STEEL SURFACES

| Test | Ti pretreatment                              | Ti treatment                                          | Anti-wear data                               | Anti-seizure data                                                       |
|------|----------------------------------------------|-------------------------------------------------------|----------------------------------------------|-------------------------------------------------------------------------|
| A1   | Toluene cleaned <sup>b</sup>                 | None                                                  | 10 kg. load—1 minute, 2-3 mm. scars          | Seized immediately.                                                     |
| A2   | do <sup>b</sup>                              | NaF immersion <sup>c</sup> for 5 hours at 650° C.     | 50 kg. load—good after 6 hours, test halted. | To 2,000 lbs. jaw load.                                                 |
| A3   | do <sup>b</sup>                              | NaF immersion <sup>c</sup> for 3 hours at 540° C.     | do                                           | 1,500 lbs. jaw load seized.                                             |
| A4   | Toluene cleaned,<br>HF pickled. <sup>d</sup> | None                                                  | 10 kg. load—1 minute, 2 mm. scars            | Welding and extreme wear on way up to 250 lbs. jaw load-torque erratic. |
| B2   | do <sup>d</sup>                              | NaF immersion <sup>c</sup> for 5 hours at 650° C.     | 50 kg. load—good after 6 hours, test halted. | Seized at 2,500 lbs. jaw load.                                          |
| B3   | do <sup>d</sup>                              | CrF <sub>3</sub> immersion                            | Balls destroyed by CrF <sub>3</sub>          |                                                                         |
| B4   | do <sup>d</sup>                              | LiF immersion <sup>c</sup> for 5 hours at 454-537° F. | Balls destroyed by LiF                       |                                                                         |

<sup>a</sup> All tests conducted using 10% by weight zinc dialkyldithiophosphate (50% by weight C<sub>8</sub> and 50% by weight C<sub>9</sub>), balance 3065 mineral oil, described in Spec. MIL-L-150168, Amendment 1, dated 10 June 1966, "Lubricating Oil, General Purpose, 100% mineral oil Except for Approved Pour-Point Depressants and Anti-Foam Agents," 100 centistokes at 75° F.

<sup>b</sup> Toluene, cleaned by degreasing in toluene.

<sup>c</sup> Titanium piece immersed in a 50 cc. porcelain crucible at room temperature, the crucible then being placed in a cool oven and brought to the stated temperature in about 1/2 hour. Piece was allowed to cool gradually after being held at the desired temperature.

<sup>d</sup> Toluene cleaned, and then pickled in a solution containing 185 ml. of 48% HF, 9 ml. concentration HNO<sub>3</sub> and the balance water to 1 liter, water washed and dried prior to immersion in NaF.

The zinc dialkyldithiophosphate may contain 100%  $C_6$  to 100%  $C_8$ , or any combination of  $C_6$ ,  $C_7$  and  $C_8$ .

From the data herein above set forth, it will become evident that the lubricity processes of the present invention improves antiwear and anti-seizure characteristics of 75A titanium pieces when rubbing at high speeds in contact with either 52100 or AISI 1137 steels when a 10% solution of zinc dialkyldithiophosphate ( $C_6$  to  $C_8$  in any proportion) is used as the lubricating agent, the balance being 3065 mineral oil.

I claim:

1. A process for improving wear and seizure resistance between rubbing titanium and steel parts comprising the steps of

immersing a cleaned titanium piece in  $NaF$  and gradually raising the temperature thereof including said titanium piece to an elevated temperature between about 540° C. and 650° C. to provide a treated piece, allowing said treated piece to cool to room temperature, and rubbing said cooled piece and said steel parts at high speeds while lubricated with a zinc dialkyldithiophosphate.

2. The process as described in claim 1 wherein said titanium piece is 75A and said steel is selected from the group consisting of 52100 and AISI 1137, said 52100 steel and said AISI 1137 steel having the following compositions:

|    | 52100     | AISI 1137 |
|----|-----------|-----------|
| C  | 0.95-1.10 | 0.32-0.39 |
| Mn | 0.25-0.45 | 1.35-1.65 |
| P  | 0.025     | 0.045     |
| S  | 0.025     |           |
| Si | 0.20-0.35 | 0.08-0.13 |
| Cr | 1.20-1.50 |           |

<sup>1</sup> Maximum.

3. The process as described in claim 1 wherein said phosphate is 10% by weight zinc dialkyldithiophosphate, the alkyl group consisting of  $C_6$  to  $C_8$  in any weight pro-

portion, balance being 3065 mineral oil having the following properties:

|    |                              |       |
|----|------------------------------|-------|
| 5  | Viscosity, SSU at 210° F.    | 60-70 |
|    | Viscosity index (min.)       | 75    |
| 5  | Pour Point, ° F. (max.)      | 5     |
|    | Flash Point, ° F. (min.)     | 410   |
| 10 | Work Factor (min.)           | 0.85  |
|    | Neutralization number (max.) | 0.10  |
| 15 | Water, percent (max.)        | None  |
|    | Ash, percent (max.)          | 0.003 |
|    | Saponification number (max.) | 0.50  |
|    | Nature of carbon             | (1)   |
|    | Total S, percent (max.)      | 0.50  |
| 20 | Precipitation number (max.)  | 0.01  |

<sup>1</sup> Loose and flakey.

4. The process as described in claim 3 wherein said cleaned titanium piece has been degreased in toluene, said elevated temperature is about 650° C. and said extended period is about 5 hours.

5. The process as described in claim 3 wherein said cleaned titanium piece has been degreased in toluene, and said extended period ranges between about 3 to 5 hours.

6. The process as described in claim 3 wherein said cleaned titanium piece has been degreased in toluene, and then pickled in a hydrofluoric acid solution, and wherein said elevated temperature is about 650° C. and said extended period is about 5 hours.

30

#### References Cited

##### UNITED STATES PATENTS

|           |           |                |            |          |
|-----------|-----------|----------------|------------|----------|
| 2,328,933 | 9/1943    | Streicher      | 148-20     |          |
| 3,041,215 | 6/1962    | Jenkins et al. | 148-6.14 R |          |
| 35        | 2,554,042 | 5/1951         | Mayfield   | 148-20 X |
|           | 3,158,515 | 11/1964        | McLael     | 148-20   |
|           | 2,844,499 | 7/1958         | Wainer     | 148-20   |
|           | 2,838,430 | 6/1958         | Argenta.   |          |

##### OTHER REFERENCES

40 40 Shapiro, ASLE Transactions 12(1), 1969, pp. 80-85.

RALPH S. KENDALL, Primary Examiner

U.S. CL. X.R.

45 117-127; 148-6.14; 308-241